

## UNITED STATES PATENT OFFICE.

WILLIAM E. FLETCHER, OF PHILADELPHIA, PENNSYLVANIA, ASSIGNOR TO ATLAS POWDER COMPANY, OF WILMINGTON, DELAWARE, A CORPORATION OF DELAWARE.

## WATERPROOF SHADE FABRIC.

No Drawing.

Application filed December 23, 1924. Serial No. 757,764.

The primary object of this invention is to produce a light weight, water-proof, crack resistant fabric, particularly adapted for use in the manufacture of window shades.

In the past it has been customary to use light weight textile materials, either sized or not, for such purposes as making window shades. In the endeavor to secure low priced products, light and flimsy fabrics such as sheeting are frequently used. These flimsy fabrics have little body and permit the passage of a large amount of light. In order to give these fabrics the necessary body, and to render them sufficiently opaque, the fabrics are sized and filled with pigments. Shades made of such sized goods are not water resistant and are easily damaged when they become wet from rain, snow or other causes. Furthermore, as the shades age, the filling material begins to crack and separate from the goods or to dust away, therefrom. This renders the shades unsightly and greatly shortens their life. The filling of the fabric with sizing and pigment tends to make the resultant product more or less brittle and this, in conjunction with the constant flexing to which the shade is subjected in use, has a tendency to cause cracking which further adds to the unsightly appearance of the shade. The process which I have devised for the treatment of materials adapted for use in the manufacture of window shades eliminates the difficulties above referred to and produces a fabric which is light enough for the use stated, is wholly waterproof, so that it will not be in the least damaged by long exposure to snow or rain, and is so flexible and elastic that it will resist cracking under prolonged flexing.

Furthermore, under the process that I have devised, the coating that is applied to render the fabric waterproof serves the further useful function of binding in place any filling previously applied to the fabric, such as sizing or pigment, and thus prevents the cracking and dusting away of the same.

Broadly stated, the invention resides in coating each side of a suitable fabric, such as sheeting, Holland shade cloth, or any other suitable, light weight, fabric with a thin film of a nitrocellulose solution. By this I mean a viscous liquid, consisting of nitrocellulose, dissolved in a suitable sol-

vent or mixture of solvents of nitrocellulose and with or without the admixture of non-solvents of nitrocellulose, vegetable oils and softeners, such as camphor, triphenylphosphate, and the like. The film of nitrocellulose solution may be applied by spraying or brushing the same upon the fabric, by passing the fabric through the solution or by applying a coating of nitrocellulose with a coating machine, such as is used in the manufacture of leather cloth. I do not wish to limit myself to the method of applying the composition containing nitrocellulose, to the fabric.

The fabric may be dyed, or not, before being treated with nitrocellulose solution, and it may be filled with pigment to give body and produce any desired color before the application of the nitrocellulose film. Upon the other hand the filling of the fabric with pigment, prior to the application of the nitrocellulose film, may be omitted, and the nitrocellulose solution itself may carry suitable dyes, pigments or other coloring material to produce any desired body or any desired color.

Since nitrocellulose solutions of the character indicated are transparent, when suitable solvents are used, it follows that my method lends itself to the production of highly ornamental effects since any desired design may be imprinted upon the shade and thereafter protected by the application of the nitrocellulose film. In other words it would be possible by means of this process to beautifully decorate the shades with delicate water colors, which would not, of themselves, be in the least resistant to moisture, nor adapted for use upon window shades, and thereafter render these effects permanent by protecting them with a transparent coating of nitrocellulose solution through which the ornamentation would be visible.

It is important in producing window shade material for the trade that the material be very light in weight and quite thin. For that reason I make the coating so thin that the total weight of the entire film will not exceed one ounce per square yard. After a film has been applied to one side of the fabric that side is dried and then the film is applied to the other side of the fabric and the second side dried.

Where a thin transparent coating of nitro-

cellulose solution is applied to shade cloths of conventional kinds, the appearance of the cloth is not materially changed.

Having described my invention, what I claim is:

As an article of manufacture, a base consisting of light-weight sized or filled fabrics, and a flexible, elastic and waterproof film

of a pyroxylin material upon each side thereof, said film being so thin that the total weight thereof does not exceed one ounce per square yard.

In testimony whereof he affixes his signature.

WILLIAM E. FLETCHER.